

Feb. 16, 1954

W. R. KEEN

2,669,001

## METHOD AND APPARATUS FOR TREATING YARNS

Filed Sept. 29, 1949



INVENTOR  
WILLIAM ROLLIN KEEN

BY *Paul J. Schmitz*  
ATTORNEY

## UNITED STATES PATENT OFFICE

2,669,001

METHOD AND APPARATUS FOR TREATING  
YARNS

William Rollin Keen, Bowling Green, Pa., assignor to Collins &amp; Sikman Corporation, Philadelphia, Pa., a corporation of Delaware

Application September 29, 1949, Serial No. 118,602

3 Claims. (Cl. 28—72)

## 1

This invention relates to a process of preparing yarns for fabrics especially pile fabrics and to apparatus for carrying out the process in a simple and practical manner. More particularly the invention is directed to the forming of configurations in and the setting of continuous strands of nylon yarn by the progressive application of distorting forces and heat followed by a subsequent heat treatment. The distorting force may be and preferably is without high pressure such as would flatten the fibers or strands being treated. By the present improvements there may be produced yarns which have an all-over or localized crimped or curled effect.

The invention is adapted to the production of nylon upholstery or floor covering pile yarns and is useful for producing yarns for other fabrics including flat fabrics.

The novel process may, if desired, be carried out concurrently with a weaving process, but is suitable for high speed mass production use and accordingly it is preferred that a single apparatus serve a number of looms.

According to the invention a supply of nylon yarns may be drawn from a source such as a spool or beam in sheet form and passes between forming members such as intermeshing sprocket- or gear-like members preferably arranged so as not to pinch the yarns to an extent to flatten individual fibers of the yarn. The function of these gear-like members is to partially set or facilitate the setting of the yarn as by heat while in the deformed position.

The deformed and partially set yarns are advanced to an apron and a heating device which sets the relaxed yarns by dry heat, steam or moist steam heat whereupon the yarn may be cooled and advanced into a pile fabric or other loom or it may be rebeamed after cooling or otherwise packaged as desired. While synthetic linear polyamide yarns may be preheated to some extent, the temperature at the deforming members will preferably be higher than that previously attained by the incoming yarns. The setting temperature will, of course, be less than required to bring fibers to the melting point of the particular fibers in the synthetic yarn. It will be noted, however, that where the heat treatment time is short that the heating unit will usually have a temperature in excess of that actually attained by the fibers in the yarn.

The process may be effected with or without the use of steam or moisture, the use of which does, however, provide some insurance against air yellowing at higher temperatures. The processed

## 2

yarn is not hardened by my process, but takes on increased crushproofing proportions and becomes more resilient. It is very suitable for the pile portion of cut or uncut pile fabrics as well as producing unusual effects in flat fabrics, all without harshening of the products.

An object of invention is to provide a deformed heat set strand of synthetic fibers such as nylon.

Another object is to provide a process and an apparatus for heat setting deformed nylon and similar untreated yarns.

Another object is to provide a process in which nylon in the form of a sheet is deformed and partially set and subsequently more permanently set.

Another object is to provide a continuous method of curling or crimping a supply of nylon yarns in side by side or sheet form.

Another object is to provide a crimping apparatus which may be conveniently set up for operation.

Another object is to provide an intermittently crimped nylon yarn which has been set at high temperatures.

These and other objects will be manifest from the following description, claims and drawing in which:

Figure 1 is a diagrammatic side elevational view of an apparatus suitable for carrying out the invention.

Figure 2 is a similar view of a modification.

Figure 3 shows an intermittently crimped yarn having crimped portions 63 and straight portions 64.

In Figure 1 a source of supply of nylon yarns 9 is carried on beam or spool 10. The yarn forms a sheet 11 of any desired number of yarns. A pair of feed rolls 12 advance the yarns from the beam which may be rotated by the feed rolls or separately driven in a convenient manner.

Gears 13, 14, 15 and 16 form a cluster, gear 13 being connected to a source of power (not shown). Gear 14 is an idler introduced so that gears 15 and 16 will be driven at the same rate when the deforming members 17 and 18 on the gear shafts 20, 21 for gears 15 and 16 are intermeshing. Preferably the intermeshing members do not operate as gears, but are driven members which contact, deform and heat the yarns to produce a partial setting without excessively squeezing the yarns. This enables deformation of the strands from a straight line without material injury to the heated fibers.

The length of time that the strands are deformed by members 17 and 18 is usually too short for a "permanent setting." In order to increase

the output I prefer to merely deform and partially set the strands while they are between the intermeshing members 17 and 18. These members may have strand contacting portions of various sizes and shapes, all of which will be referred to as teeth 19 irrespective of their exact shape. The teeth 19 may be conveniently heated as by resistance heating units (not shown) or by high frequency induction units or the like.

The shaft 20 is fixed, whereas shaft 21 is mounted at one end on arm 22 of bellcrank 23 for pivotal movement about shaft 24 on which gear 13 is mounted. A follower 25 on bellcrank 23 engages cam 26 on shaft 27. A clutch 28 may cut quick acting cam 26 into and out of rotating operation. The result is that when cam 26 is in the position shown in Figure 1 and not rotating, the heated members 17 and 18 will continuously crimp and partially set yarn moving through. When the clutch 28 is cut in the cam 26 will rotate and quickly separate the teeth of deforming members 17 and 18. Simultaneously the gear 16 will move along gear 13 and the sheet 11 will be advanced through the device without being crimped. When member 17 and gear 16 are returned to intermeshing position, they will be in synchronism as before. It will thus be seen that the devices may produce continuously or intermittently crimped yarns with sharply defined zones.

After crimping the sheet 11 moves partly by gravity to a preferably inclined apron 30 of material resistant to the effects of heat such as metal or specially prepared fabric which withstands high temperatures. Coated cotton fabrics known per se may be used. The apron 30 passes about cylinders 31 and 32 and may be driven as by a nip formed by cylinders 33 and 34.

The object of the apron 30 being inclined is to maintain as far as possible the initial deformation of the relaxed strands. The final setting may be by steam or dry heat or combination of both.

In Figure 1 moisture in the form of steam or a fine spray of water may be introduced through conduit 34 on to the fibers prior to their entering heating unit 35 for the final setting at a temperature usually as high or higher than the partial setting. Moisture may be added and may be heated to steam in the unit or it may be dispensed with in some cases.

The final set yarns or strands are advanced to a second inclined apron 36 mounted on and driven by cylinders 37, 38 and 39 as shown. They are cooled as by a water spray or cool air current from conduit 42 so as to be prepared for removal by rolls 40, 41 and used or packaged as desired.

The melting point of much of the commercially available nylon is in the neighborhood of 480° F. and tackiness or sticking occurs at about 360° F. The setting properties of nylon are not fully understood, the factor in or character of the fiber which gives nylon some of its setting properties being sometimes referred to as element X. According to the present improvement, it is feasible to deform and set yarn at high temperatures including those well into the range where sticking occurs. Temperatures from 300° F. to 440° F. are preferred because at these temperatures the time of contact may be quite short and still produce a partial setting. Such stickiness as may be induced during processing does not usually appear to cause the fibers to adhere to each other after cooling.

It should also be noted that in intermittently deformed yarns, Figure 3, the twist in straight

portions as well as in the deformed portion may be set. Portions not deformed may be subjected to setting heat either as the yarns pass freely between the crimping cylinders 17 and 18 or subsequently as described.

If the deforming apparatus and control cam 26 is operating slowly a permanently set crimp may be introduced and the straight portions remain unheated at this stage of the process. These seemingly inconsistent results are effected by choice of setting temperatures used, the speed of the apparatus and the distance of the deforming rolls from one another or the strand.

Broadly then the crimping rolls Figure 1 are sources of heat which by quick movement into and out of setting position and with or without strand pressure may give a variety of results.

A twisted synthetic yarn having alternate straight and deformed heat set portions is believed to be distinctly new and will produce different effects in fabrics than the intermittently set prior art yarns such as mohair.

In Figure 2 a beam 50 having a supply of twisted nylon yarns similar to 9 is rotatable and the yarns advanced by cylinders 51, 52 as before. The yarns may be wet by a spray through 53.

After leaving cylinders 51, 52 the yarns pass about rods 54 which may vary in number and be of the same or gradually decreasing diameters as shown. The rods are all driven in the same direction and the yarns contact approximately the entire periphery of each rod. Each strand passes entirely around the first rod and then over to and about the second rod and so on. The rods 54 are quite small usually varying in size from  $\frac{1}{4}$  inch diameter downward and may be of such material as may be maintained at a constant temperature in a manner known per se. Alternate rods 54 may be driven from gears (not shown) on each side so all have the same direction of rotation as will be understood.

As in Figure 1, after partial setting, the yarns may be sprayed or not at 55 prior to entering heat chamber 56 on apron assembly 57 for final setting. The yarn is then advanced and sprayed or otherwise cooled before strong tensions are applied. The apron 58 on rolls 59, 60 driven by 59 and 61 are preferably slightly inclined to better maintain control of the strands. Water or cool air may be introduced at 62.

The two illustrated embodiments depict continuous processing and are preferred because of the uniformity of results obtainable. It is, however, practical to deposit the partially set deformed yarns in a can or other supporting container without tension and transfer the container to an autoclave or steam chest to complete the setting of the yarns under controlled conditions of dry heat or steam pressure and temperature. The container support may cause additional deformations because of the packing or weight of the strands on each other. After final heat setting the strands or yarns will be cooled. The cooling here and in the continuous process embodiments may be by removal from the high temperature zone and some delay prior to use or packaging.

Referring again to Figure 1 it will be noted that both aprons are preferably inclined and that apron 39 is positioned close to the crimping mechanism to minimize the effect of the yarns' own weight. The mechanism may be so rearranged that the strand is received by the support

almost immediately after the strand leaves a crimping member.

The apparatus of Figure 2 may also be arranged for downward flow of the processed strands if desired.

The action of pattern cam 26 and associated parts aside from their operating functions, facilitates the setting up of the device for operation by allowing free ends of a supply to be readily introduced. This, together with the gravity feed, provides advantage with respect to entanglement of separate yarns which is a substantial practical problem in the handling of conventional nylon yarns. By the present improvement proper spacing can readily be maintained in the setting up operation with out the use of stiffening materials, resins, size or the like. In both the continuous and container support described embodiments the strands are finally set while in a nearly tensionless condition. The tension caused by the weight of short lengths of the yarn is overcome by the partial setting.

Having described my invention in connection with preferred embodiments, but not wishing to be expressly limited thereto, I claim:

1. In a process for deforming a twisted nylon ply yarn at intervals along its length, the steps which consist of leading the nylon yarn forwardly from a supply, passing the yarn through intermeshing driven gear-shaped members, heating the gear-shaped members to a temperature in the range from 300° F. to 440° F., intermittently disengaging and then reengaging said gear-shaped members while continuing to lead said yarn forwardly, thereby leaving deformed portions in said yarn separated by straight portions, applying heat to both the deformed and straight portions while said yarn is in motion and not under tension, thereby setting the deformed portions and the straight portions, and then cooling the yarn.

2. The invention of claim 1 further characterized by the step of supplying heat to said yarn during the periods of disengagement of the heated gear-shaped members.

3. In a process for deforming a twisted nylon

ply yarn at intervals along its length, the steps which consist of leading the nylon yarn forwardly from a supply, passing the yarn through intermeshing driven gear-shaped members, heating the gear-shaped members to a temperature in the range from 300° F. to 440° F., intermittently disengaging and then reengaging said gear-shaped members while continuing to lead said yarn forwardly, thereby leaving deformed portions in said yarn separated by straight portions, transferring the deformed yarn through a support, moving the support upwardly and simultaneously applying heat to the yarn while it is supported substantially without tension and then cooling the yarn while it is in motion and not under tension.

WILLIAM ROLLIN KEEN.

References Cited in the file of this patent

UNITED STATES PATENTS

|    | Number    | Name              | Date          |
|----|-----------|-------------------|---------------|
| 20 | 2,058,948 | Blumenthal et al. | Oct. 27, 1936 |
|    | 2,090,669 | Dreyfus et al.    | Aug. 24, 1937 |
|    | 2,157,117 | Miles             | May 9, 1939   |
| 25 | 2,157,118 | Heckert           | May 9, 1939   |
|    | 2,197,896 | Miles             | Apr. 23, 1940 |
|    | 2,230,272 | Slayer            | Feb. 4, 1941  |
|    | 2,278,879 | Hunter            | Apr. 7, 1942  |
|    | 2,303,476 | Zu Kornegg        | Dec. 1, 1942  |
| 30 | 2,321,757 | Lodge             | June 15, 1943 |
|    | 2,369,395 | Heymann           | Feb. 13, 1945 |
|    | 2,390,572 | De Brabander      | Dec. 11, 1945 |
|    | 2,394,165 | Getaz             | Feb. 5, 1946  |
|    | 2,401,389 | Truitt            | June 4, 1946  |
| 35 | 2,440,209 | Redman            | Apr. 20, 1948 |
|    | 2,459,620 | Cleeland et al.   | Jan. 18, 1949 |
|    | 2,483,861 | Weiss             | Oct. 4, 1949  |
|    | 2,493,830 | Picard            | Jan. 10, 1950 |

FOREIGN PATENTS

|    | Number  | Country       | Date          |
|----|---------|---------------|---------------|
| 40 | 451,102 | Great Britain | July 24, 1936 |
|    | 558,297 | Great Britain | Dec. 30, 1943 |
|    | 702,227 | Germany       | Feb. 3, 1941  |